

# UNITED STATES PATENT OFFICE.

ALBERT E. GARRETT, OF ST. ALBANS, ENGLAND.

## TREATMENT OF WOOLEN GOODS.

1,147,011.

Specification of Letters Patent. Patented July 20, 1915.

No Drawing.

Application filed October 6, 1914. Serial No. 865,366.

*To all whom it may concern:*

Be it known that I, ALBERT EDWARD GARRETT, a subject of the King of Great Britain, and resident of Yaverland, Clarence Road, 5 St. Albans, in the county of Hertford, England, have invented certain new and useful Improvements in the Treatment of Woolen Goods, of which the following is a specification.

10 This invention relates to the finishing of woolen materials such as are used for under-garments, shirts and the like. Such woolen materials are very frequently subjected to chemical processes for the reduction of their 15 tendency to shrink when washed. The processes in question are well known involving some form of chlorination of the wool and will be referred to hereinafter as the treatment in the chlorin bath. The chlorin in 20 the bath acts as an oxidizing agent as is well known. After treatment in the bath, the goods are usually passed through a clearing bath containing substances such as antichlor for removing any excess of the chlorin used 25 in the chlorin bath. After this treatment the goods will not shrink to any considerable extent when in use, but they are open to the great objection that they will absorb moisture very much more readily than untreated 30 materials.

It is the object of the present invention to provide a process which will make it possible for goods, after treatment in the chlorin bath, to be rendered substantially as 35 good as untreated materials in regard to their behavior in resisting the absorption of moisture. For this purpose the goods, directly after the treatment in the chlorin bath, or after further treatment (when such 40 is applied) in the clearing bath containing antichlor or the like, are rinsed with water as thoroughly and as quickly as possible in order to remove all traces of the chemicals used, and are then submitted to immersion 45 for a few minutes in a bath containing a comparatively weak solution of soap and ammonia at a convenient temperature, preferably not exceeding 50° C. The strength of this bath is a matter of great importance, 50 and a pure soap should be used which is free from alkali. Usually a rather weak soap-solution is employed, containing as a minimum about 4 or 5 cubic centimeters, and as a maximum from 10 to 15 cubic centimeters 55 of strong (.880) ammonia per liter, while about one liter is used for each 60 grams of

the fabric. If any considerably larger proportion of ammonia per liter were used, the material would be spoiled. The goods may next be scoured with soap solution or not, 60 as may be considered preferable, and are rinsed thoroughly in water in order to clear them. Finally they are dried and finished by pressing. If white goods are to be produced the bleaching process should be an 65 oxidizing one, carried out with a peroxid, such as H<sub>2</sub>O<sub>2</sub> or a metallic peroxid, and this must not be applied before the treatment in the chlorin bath as is usual, but must be applied after the rinsing which follows the 70 ammonia-soap bath, the goods being finally rinsed thoroughly and then dried and finished.

The invention is not limited in its application to woolen fabrics or garments already 75 made, but it may be applied also to the wool before the spinning or to the yarn, and the process may be used for the purpose of rendering finished goods which have been treated only in the usual chlorin bath, more re- 80 sistant to moisture.

The following examples will indicate how the process is carried out in practice. It is assumed that the goods are treated in lots each of about 50 lbs. weight. 85

When woolen goods in natural color are to be treated, they are usually first scoured thoroughly, milled and then submitted to the chlorin bath, the strength of which will vary according to the nature of the material. 90 The chlorin bath treatment is well known and will require no further explanation here. The goods are now rinsed thoroughly in water, and may then be submitted at once to the ammonia-soap bath. A suitable 95 strength of this for 50 lbs. of material to be treated is as follows:—6 lbs. of soap which is as free as possible from alkali, 5 pints of strong ammonia (.880 sp. gr.) and 120 gallons of water. After about 5 minutes im- 100 mersion in the ammonia-soap bath at say 50° C., the goods are withdrawn, scoured or not as may be preferred with soap solution, rinsed very thoroughly in water to clear them, and finally dried and finished by usual 105 methods.

Sometimes it may be desirable to subject the goods to a longer treatment in the ammonia-soap bath; either up to say 10 minutes in the same solution, or, preferably, in 110 two or more stages of say 5 minutes each, with a rinsing operation between, a fresh am-

monia-soap bath being used for each period of immersion. For most goods, however, a single immersion is quite sufficient to leave the goods in the desired condition, particularly if the chlorin bath was not too strong and if the rinsing following upon it was thorough. The treatment in the clearing bath containing antichlor also seems to be unnecessary if the rinsing is thorough, but after imperfect rinsing the chemical reagents which remain in the goods may largely neutralize the action of the ammonia-soap bath. The final rinsing or washing also must be effected as quickly as possible and must be thorough in order that all traces of the ammonia-soap solution may be removed.

If white goods are to be produced, the treatment is identical down to the stage of rinsing after the ammonia-soap bath, but after that the goods are bleached by peroxid applied in one of the known ways, are rinsed again thoroughly thereafter, and finally dried and finished.

All goods treated by the process above set forth, whether bleached or not, are remarkably resistant to moisture, that is to say they absorb moisture only very slowly. The process therefore enables woolen goods to be produced which combine the advantage of resistance to shrinkage with the retention of the normal behavior of wool toward moisture.

In applying the process to goods which are supposed to have been finished already, but have only been treated in the chlorin bath, these are washed and then subjected to the ammonia-soap bath treatment as hereinbefore set forth, but they are liable to require longer treatment or a stronger ammonia solution, or more than one immersion in the ammonia-soap bath. This method of working is only to be adopted therefore as a remedy for otherwise defective goods, and would not be adopted by preference if it were possible to carry out the process in successive stages as set out above.

In applying the process to wool or to yarn before these are made up into fabrics, substantially the same operations are performed, but the ammonia-soap solution will preferably not contain more than about 5 cubic centimeters of ammonia per liter of the solution.

Having thus described my invention what I claim as new and desire to secure by Letters Patent is:—

1. Process for treating woolen material

consisting in submitting the material to the action of a chlorin bath, and subsequently submitting the material to the action of a weak ammonia-soap solution.

2. Process for treating woolen material consisting in submitting the material to the action of a chlorin bath, rinsing the material and then submitting it to the action of a weak ammonia-soap solution and finally rinsing, drying and finishing the material.

3. Process for treating woolen material which has been subjected to treatment in a chlorin bath, the process consisting in submitting the material to the action of a weak ammonia-soap solution and finally rinsing and drying the material.

4. Process for treating woolen material consisting in submitting the material to the action of a chlorin bath, and subsequently submitting the material to the action of a weak ammonia-soap solution containing not more than 15 cubic centimeters of strong ammonia per liter of the soap solution.

5. Process for treating woolen material consisting in submitting the material to chlorination in a chlorin bath, rinsing the material, submitting it to the treatment in an ammonia-soap bath containing not more than 15 cubic centimeters of strong ammonia per liter, the treatment in the said bath lasting approximately five minutes, subsequently rinsing the material thoroughly and finally drying and finishing the same.

6. Process for treating woolen material which has been subjected to treatment in a chlorin bath, the process consisting in submitting the material to the action of a weak ammonia-soap solution containing not more than 15 cubic centimeters of strong ammonia per liter, the treatment in the said bath lasting approximately five minutes, subsequently rinsing the material thoroughly and finally drying and finishing the same.

7. As a new article of manufacture, woolen material which has been chlorinated and subsequently treated with a weak ammonia-soap solution, whereby it is rendered resistant to shrinkage and repellent to water which it will only absorb very slowly.

In witness whereof I have hereunto signed my name this 24th day of September 1914 in the presence of two subscribing witnesses.

ALBERT E. GARRETT.

Witnesses:

HUBERT A. GILL,  
H. D. JAMESON.